

## UNITED STATES PATENT OFFICE

1,935,263

## TREATMENT OF FABRICS

George Holland Ellis, Spondon, near Derby, England, assignor to Celanese Corporation of America, a corporation of Delaware

No Drawing. Application December 3, 1926,  
Serial No. 152,516, and in Great Britain July  
27, 1926

7 Claims. (Cl. 8—20)

This invention relates to the treatment of woven, knitted or other fabrics—made with or containing threads or yarns composed of or comprising filaments or fibres of cellulose acetate or other esters or ethers of cellulose,—for the purpose of rendering them less liable to or immune from development of faults caused through lack of cohesion or low coefficient of friction existing between the threads or yarns of the fabrics at their points of crossing or interlooping.

In the case of woven fabrics these faults are commonly referred to as "slipping", the term indicating that stresses in usage or in processes subsequent to weaving cause the threads of one component (i. e. the warp or weft) to slip over those of the other and produce, at the point of slipping, uneven distribution of the warp threads or weft threads. The fault is least observable in closely woven fabrics having a high number of reed and pick and is most likely to occur in fabrics with a small number of crossings (i. e. points of contact of warp and weft) per unit area.

In the case of circular knitted fabrics or other weft-knitted fabrics the fault is commonly known as "laddering" and is caused by a line or series of loops in the fabric (on breakage of a loop or thread) becoming drawn out of or slipping out of the adjacent loops through which they are threaded in the structure of the fabric, owing to lack of cohesion or low coefficient of friction at the points of contact of the loops, so that a ladder-like defect results; while in the case of warp-knitted fabrics the fault is commonly known as "splitting" and is produced by the fabric "splitting" continuously along a wale of the fabric, without tearing, if a cut happens to be made lengthwise in the middle of the wale in a direction towards the beginning of the fabric, such splitting being likewise due to lack of cohesion or low coefficient of friction existing between the threads of the fabric.

It has now been found that by subjecting woven, knitted or other fabrics,—and especially fabrics made with or containing threads or yarns composed of or comprising filaments or fibres of cellulose acetate or other esters or cellulose ethers—to the process of the present invention, their tendency to develop the faults of the character referred to is greatly minimized or even eliminated.

The precise reason for the efficacy of the process of the present invention is not entirely clear, but it appears in general to be due to physical modification of the yarns by which they

are swollen out, either by actual swelling or increase of volume of the filament or fibre unit itself or by penetration of the interstices between the filaments, or both, so that the binding power of the threads or yarns is increased producing a more resistant fabric.

According to the present invention for the purpose referred to woven, knitted or other fabrics,—made with or containing yarns or threads composed of or comprising filaments or fibres of cellulose acetate, or other esters or ethers of cellulose,—are subjected to simple or repeated application by impregnation with one or more substances or agents having a swelling action upon the fibres of the fabrics. Such substances or agents are chiefly organic bodies. The process of the present application is carried out with such substances or agents and in such a manner that merely an increase of the cohesion and of the coefficient of friction between the yarn or threads of the treated material is produced and no solution of the cellulose derivative takes place which would cause adhesion between the yarns or threads.

Examples of the substances or agents which I may use for the purpose of the invention, and which are especially useful for the treatment of fabrics made with or containing cellulose acetate threads or fibres are:—

(a) Hydrocarbons such as those, of the paraffin, aromatic, naphthene or terpene series, and their hydrogenated and halogenated derivatives for example; hexane, decane, dodecane, or higher paraffin hydrocarbons or mixtures of such as may occur in various commercial liquids of paraffin like gasoline, and the like; benzene, toluene, xylenes, naphthalenes, dekanaphthene, undekanaphthene, dodekanaphthene, pinene, sylvestrene; hexahydrobenzene, tetrahydronaphthalene, trichlorethylene, tetrachlorethane, chlor or polychlor benzenes, chlor or polychlor toluenes, chlor or polychlor xylenes; alphachlornaphthalene, betachlornaphthalene, polychlornaphthalenes.

(b) Alcoholic and phenolic bodies of the various chemical series, and their halogenated or hydrogenated derivatives, for instance, ethyl alcohol, propylalcohol, glycerol, phenol, cresols, xylenols, hexahydrophenol, alphanaphthol, betanaphthol, resorcin, catechol, guaiacol, anisol, tetrahydronaphthol, chlorhydrin, chlorphenol, chlornaphthols.

(c) Amino compounds, or their hydroxy or halogenated derivatives for instance aniline, alkyl- or dialkylanilines, alkyl or dialkyl tolui-

dines, alkyl or dialkyl xylidines, benzylaniline, diphenylamine, naphthylamines, alkyl and aryl naphthylamines such as phenyl- and ethyl-alphanaphthylamines, chloranilines, chlornaphthylamines, aminophenols, aminonaphthols, alkylaminophenols, alkylaminonaphthols.

(d) Ketonic, aldehydic and miscellaneous organic substances such as acetone, diacetonealcohol, formaldehyde, benzaldehyde, and nitro derivatives such as nitrobenzene, nitrotoluene and the like.

The bodies or agents having a swelling action may be applied to the goods in any suitable manner, at any suitable temperatures or pressures. 15 By way of example, they may be applied by any of the following methods, it being understood that I in no wise limit myself in this respect:—

(1) The selected agent or mixture of agents may be applied as such where feasible, as in 20 the case of liquids such as benzene, toluene, turpentine, and the like.

(2) The agent or mixture of agents may be applied in solution or admixture with indifferent solvents or liquids, as for instance, benzaldehyde 25 in solution or mixed with diethylether, phenol or ethylalcohol in water.

(3) The agent or mixture of agents, where insoluble or insufficiently soluble in or miscible with water may be applied in colloidal dispersion 30 in aqueous media.

Such colloidal dispersions may be formed by any methods known in the colloidal arts, but in particular they may be formed by or with the aid of the methods described in prior British 35 specifications Nos. 219,349, 224,925, 242,393, 9503/26, or 273,819 or 273,820, and in U. S. Patents Nos. 1,618,413, 1,618,414, 1,694,413 or 1,840,572, by treating the swelling agents with one or more of the solubilizing agents of the said 40 specifications which treatment may be in presence or absence of water, (or in presence of larger quantities of water with subsequent concentration or drying), heating if necessary and diluting the solubilized or dispersed modifications 45 so formed or, as required. The solubilizing agents of the prior British specification No. 219,349 and U. S. Patent No. 1,618,413, are as therein stated sulphoricinoleic or other sulphated fatty acids or other bodies having oily or fatty 50 characteristics, namely higher fatty acids or sulphonated or other derivatives thereof containing salt-forming groups or salts of such acids or bodies, for instance their alkali or ammonium salts, or a mixture of two or more of such acids 55 or bodies and salts, and the said British specification No. 219,349, and U. S. Patent No. 1,618,413, mentions as examples of such solubilizing agents oleic, stearic, palmitic, sulphoricinoleic, their alkali or ammonium salts, mixtures of such acids, 60 and mixtures of such acids and salts.

The solubilizing agents of the said British specification No. 224,925 and U. S. Patent No. 1,618,414 are, as therein stated, carbocyclic compounds containing in their structure one or more 65 salt forming groups or sodium or other salts of said compounds, or mixtures of one or more thereof with one or more of the solubilizing agents of the British specification No. 219,349 and U. S. Patent No. 1,618,413; and as examples of such 70 carbocyclic compounds or their salts British specification No. 224,925 and U. S. Patent No. 1,618,414 mention naphthenic acids, naphthene sulphonic acids or other carboxylic or sulphonic acids of the cyclo paraffins, phenols, sulphonic 75 acids, carboxylic acids, phenolsulphonic acids or

other derivatives of the benzene, naphthalene or anthracene series, or other derivatives of saturated or non-saturated cyclic hydrocarbons containing one or more salt forming groups, or sodium or other salts of such bodies. The solubilizing agents 80 of our said previous British specification No. 242,393 and U. S. Patent No. 1,694,413 are, as therein stated one or more sulphoaromatic fatty acids such as sulphobenzenestearic acid (Twitchell reagent) or derivatives thereof such as sulphophenol-stearic acid, sulphonaphthalene stearic acid, or salts of such bodies. The solubilizing agents of our said previous British specification No. 273,819 and U. S. Patent No. 1,840,572 are, as 85 therein stated, sulphoaromatic ricinoleic acids or salts thereof, for instance sulphobenzene ricinoleic acid, sulphophenol ricinoleic acid or sulphonaphthalene ricinoleic acids or their alkali or ammonium salts. The solubilizing agents of our prior British specification No. 273,820 are, as 90 therein stated, soluble resin soaps or sodium or other soluble salts or soaps of resin acids.

The application of the swelling agents in the form of their colloidal dispersions—and especially in form of their colloidal dispersions prepared by 100 the methods described in our previous specifications—is particularly useful from a commercial point of view in view of the ease and safety of manipulation and economy. Further, many of the solubilizing agents of our said previous specifications when employed for preparing the aqueous dispersions for practising the present invention, produce liquids of low surface tension and can contribute materially to the efficacy of the process since liquids of low surface tension penetrate or wet out better and thus the interstices between the filaments tend to become penetrated more readily, which is a material aid.

Examples of such colloidal dispersions which I have found particularly useful for the purpose 115 of the present invention are dispersions of xylene in Turkey red oil, dispersions of nitrobenzene in concentrated soap solutions, dispersions of solvent naphtha in concentrated soap solutions, dispersions of xylene in aqueous sulphoricinoleic 120 acid and the like.

When it is desired to perform the process of the present invention by the methods 1 or 2, a closed extraction apparatus will usually be used since most of the impregnating substances of the present invention are inflammable or volatile. For method 3 (application in form of colloidal dispersions in aqueous media) ordinary dyeing, scouring or impregnation machinery is available such as the jigger, winch or reel machine, open 125 soaper, beam dyeing machine and the like familiar in these trades. In all methods of application temperatures and pressures will be chosen to suit the individual conditions and agents employed but usually the process of the present invention 130 is more efficacious at warm or hot temperatures than cold. The duration may also be greatly varied according to individual circumstances and the process may be applied in continuous manner depending upon various controlling factors such 135 as the resistances of the fabric to manipulation. Further in some cases it is advantageous, when possible, to allow the agent after impregnation to remain in the fabrics for some time before removing them, for instance the impregnated fabrics 140 may be piled or rolled up and left overnight. When the treatment has been given for the requisite length of time the goods may be washed, soaped and dried and finished as desired.

The following examples illustrate the inven- 145

tion, but it is of course to be understood that they are in no way limitative.

*Example 1*

5 A fabric woven from cellulose acetate yarns is treated with boiling toluene for 3 hours in a suitable closed apparatus, for instance, an apparatus of the Soxhlet types. The fabric is thereafter removed, dried, and finished as required.

10 *Example 2*

A woven or knitted fabric of cellulose acetate yarns is treated for 1 hour at about 80° C. in a bath containing about 50 times the weight of the 15 goods of a liquor consisting of equal volumes of methylated spirit and water. At the end of this time the fabric is removed and dried without rinsing. The results may be improved by two successive after treatments at 60° C. in baths containing about 2.5 grams per litre of a good textile soap, followed by rinsing two or three times in warm soft water to remove excess of soap. The 20 first wash water may advantageously contain a little ammonia. The fabric is afterwards dried 25 and finished as desired.

*Example 3*

A woven or knitted fabric of cellulose acetate is treated in the cold for 1 hour in about 40 times 30 its weight of an aqueous solution of phenol containing approximately 1.5 grams per litre. After this treatment the fabric is removed, rinsed, and dried until the smell of phenol no longer remains. As in Example 2 improved results may 35 be obtained by a subsequent double soaping followed by adequate rinsing.

*Example 4*

A woven or knitted fabric of cellulose acetate 40 yarn is treated at 80° C. in any suitable manner, but preferably by means of an ordinary padding mangle, with a dispersion containing: 1 part by volume of xylene and 9 parts by volume of Turkey red oil (50% fatty acids). The pressure is so 45 adjusted that the fabric retains about 85% of its weight of the dispersion. The operation may be continuous and after the impregnation and squeeze the goods are preferably rolled up to maintain the temperature and left for a time. 50 The efficacy of the treatment is dependent upon the time factor and it is found desirable in practice to leave the goods overnight. They are then scoured at 60° C. with a soap solution containing 2.5 grams per litre and afterwards washed 55 with warm soft water, which may contain a little ammonia if desired, until free from the agents used. The whole process may then be repeated

to obtain a considerable improvement of the result. The goods may afterwards be subjected to dyeing operations or other treatments as desired.

What I claim and desire to secure by Letters Patent is:—

1. Process for the treatment of fabrics containing organic substitution derivatives of cellulose to render them less liable to develop faults, comprising impregnating the fabrics with substances capable of swelling, without dissolving, the cellulose derivatives so as to increase the cohesion and coefficient of friction between the yarns of said fabric.

2. Process for the treatment of fabrics containing organic substitution derivatives of cellulose to render them less liable to develop faults, comprising impregnating the fabrics with aqueous colloidal solutions of substances capable of swelling, without dissolving, the cellulose derivative 95 so as to increase the cohesion and coefficient of friction between the yarns of said fabric.

3. Process for the treatment of fabrics containing cellulose acetate to render them less liable to develop faults, comprising impregnating the 100 fabrics with substances capable of swelling, without dissolving, the cellulose acetate so as to increase the cohesion and coefficient of friction between the yarns of said fabric.

4. Process for the treatment of fabrics containing cellulose acetate to render them less liable to develop faults, comprising impregnating the fabrics with aqueous colloidal solutions of substances capable of swelling, without dissolving, the cellulose acetate so as to increase the cohesion 105 and coefficient of friction between the yarns of said fabric.

5. Process for the treatment of fabrics comprising cellulose acetate to render them less liable to develop faults, comprising treating the fabrics 115 with aqueous colloidal solutions comprising xylene and a soap, batching the same and then scouring.

6. Process for the treatment of fabrics comprising cellulose acetate to render them less liable to develop faults, comprising treating the fabrics with aqueous colloidal solutions comprising commercial solvent naphtha and a soap, batching the 120 same and then scouring.

7. Process for the treatment of fabrics comprising cellulose acetate to render them less liable to develop faults, comprising treating the fabrics with aqueous colloidal solutions, comprising xylene and a sulphonated soap, batching the same and then scouring.

GEORGE HOLLAND ELLIS. 125

60

135

65

140

70

145

75

150

**CERTIFICATE OF CORRECTION.**

**Patent No. 1,935,263.**

**November 14, 1933.**

**GEORGE HOLLAND ELLIS.**

**It is hereby certified that error appears in the printed specification of the above numbered patent requiring correction as follows: Page 2, line 36, strike out the numerals and word "9503/26, or"; and that the said Letters Patent should be read with this correction therein that the same may conform to the record of the case in the Patent Office.**

**Signed and sealed this 19th day of December, A. D. 1933.**

**(Seal)**

**Richard Spencer  
Acting Commissioner of Patents.**